# EUROPEAN PATENT SPECIFICATION

(11) **EP 0 633 339 B1**
(45) Date of publication and mention of the grant of the patent: **26.09.2001**
(21) Application number: 94115971.7
(22) Date of filing: 07.06.1990
(51) Int. Cl.: D01D 5/098, D04H 1/56, D01D 4/02

(54) **Process and apparatus for forming fibers**
Verfahren und Anlage für Fasern-Bildung
Procédé et appareil pour la formation de fibres

(30) Priority: 07.06.1989 US 362737
(43) Date of publication of application: 11.01.1995
(62) Divisional of application: 90110818.3
(73) Proprietor: KIMBERLY-CLARK WORLDWIDE, INC., Neenah, Wisconsin 54956 (US)
(72) Inventor: Dodge, Richard N. II, Roswell, GA 30076 (US); Allen, Martin A., Dawsonville, GA 30534 (US); Wagner, Ann L., Cumming, GA 30131 (US); Fetcko, John T. III, Dawsonville, GA 30535 (US); Fowler, Larry C., Duluth, GA 30136 (US)
(74) Representative: Diehl, Hermann, Dr. Dipl.-Phys.

(56) References cited:
- EP-A- 0 293 065
- GB-A- 1 478 800
- US-A- 2 571 457
- US-A- 3 716 318
- US-A- 3 825 280
- US-A- 4 185 981
- US-A- 4 295 809
- US-A- 4 692 371
- US-A- 4 785 996

## Description

The manufacture of nonwoven fabrics is a highly developed art. Generally, nonwoven webs or mats are made by forming filaments or fibers of varying or specific diameter and depositing them on a carrier in such a manner so as to cause the filaments or fibers to overlap or entangle as a web of a desired basis weight.

Various means have been developed in an attempt to control the form of the processed fibers which in turn affects the properties of the formed web. For example, U.S. Patent 2,571,457 to Ladisch, issued October 16, 1951 discloses a spray nozzle for forming filaments and/or fibers in diameters of about one micron and smaller by passing a polymer stream through the central orifice of a nozzle with an elastic fluid such as air being caused to spiral towards the vertex of a cone. U.S. Patent 3,017,664 to Ladisch, issued January 23, 1962 discloses a fiber forming nozzle wherein a stream of polymer material exits a nozzle orifice in the form of a tube, formation of the tube being caused by the spreading of the polymer over the outside wall of a circular body positioned in the orifice. An elastic fluid rotating in a spiraling manner around the film of polymer with a very high velocity creates a vacuum between the film and elastic fluid. Fibers are picked up from the film of fiber forming liquid and drawn out to fineness in the elastic fluid. Although both Ladisch patents disclose a spiraling air which surrounds the resin flow from an orifice, the emitted air is transmitted through nozzle openings which do not surround the polymer stream.

U. S. Patent 3,543,332 to Wagner et al, issued December 1, 1970, discloses the production of fibers utilizing a spinning nozzle, the spinning nozzle having a central orifice for forming a polymer stream and additional orifices surrounding the central orifice for the passage of fiber forming air.

U. S. Patent 3,755,527 to Keller et al, issued August 28, 1973, discloses a process for producing meltblown nonwoven synthetic polymer mats. The meltblown process utilizes a plurality of extrusion orifices through which a melted polymer resin is extruded. On each side of the plurality of orifices is a hot air slot for supplying a stream of hot gas in the form of a sheet on each side of the plurality of fiber streams formed from the resin. To produce fibers having diameters between 10 and 40 µm combinations of die tip temperature, resin flow rate, and resin molecular weight are selected to give an apparent viscosity in the die holes from about 10 to 800 poise.* The viscosity is then adjusted into an operable range by varying the die tip temperature.

U. S. Patent 3,905,734 to Blair, issued September 16, 1975 discloses improvements for an apparatus for continuous tube forming by meltblowing techniques. The assembly utilizes knife-like streams of forming gas on each sideof a polymer exit orifice.

U.S. Patent No. 3,978,185 to Buntin et al, issued August 31, 1976 discloses a meltblown nonwoven mat prepared from thermoplastic polymer fibers which are alleged to be substantially completely free of polymer shot and produced at a high polymer throughput rate in a specific meltblowing process in which thermoplastic
*1 poise = 100 mPa.s
polymer resins having a specific viscosity range are degraded in the presence of a free radical source compound.

U.S. Patent Nos. to Oshido et al, 4,135,903 issued January 23, 1979 and 4,185,981 issued January 29, 1980 disclose a method and apparatus for producing fibers from a heat softening material utilizing high speed gas streams which cause the melted polymer to rotate around its central axis line and transform it into a substantially conical shape whose cross-section gradually decreases towards its flowing direction in a first cone and is caused to advance in the form of fiber from the tip of the cone in the flowing direction and outwardly in the radial direction in a second cone.

Patent EP 0293 065 discloses a method and apparatus of controlling the generation of viscous fluid fibres, droplets and combinations of the same, including hot melt adhesive and other fluids, that comprises, spraying a stream of such pressurized fluid through a fine orifice and along a predetermined direction in free flight, and simultaneously funneling a cone of pressurized air against the stream, intersecting the same in its free flight below the orifice to control the nature, dimensions and pattern of the resulting fluid coating on surfaces disposed therebelow.

It remains desirable to develop further method and apparatus for forming fibers from molten fiber forming resins suitable for then forming mats from the formed fibers wherein the apparatus and process provide increased throughput on a per-hole basis and wider operating ranges.

This object is solved by the process of independent claim 1 and the apparatus according to independent claim 14. Further advantageous features of the invention are evident from the dependent claims, the following description, examples and drawings. Further details of these uses are evident from the description and drawings. The claims are understood to be a first non-limiting approach of defining the invention in general terms.

The invention provides means for manufacturing nonwoven fabrics useful for a wide variety of applications, such as for personal care products, household cleaning materials and wipers, and the like. More specifically, the present invention provides a novel method and means for forming fibers from a fiber forming thermoplastic polymer resin suitable for forming a nonwoven web.

Apparatus and processes described in the above references are quite capable of forming flat mats or webs of nonwoven material which are most commonly subjected to additional processing for incorporation into other products such as diapers and other personal care items or subsequent conversion into such items as disposable workwear. With the advancement of nonwoven fiber forming technology, however, the uses and applications for such materials have been greatly enhanced and as new uses and applications are found, the design limitations of current equipment become more evident. Further, with the increasing costs of the polymers used in the formation of fibers, overall production costs become an ever important factor. The invention provides one way to reduce the cost of the nonwoven material by allowing to increase the production capability of the equipment, while with current meltblowing equipment, there are severe limitations as to the amount of polymer throughput which can be tolerated by the meltblowing dies. (As polymer viscosities and pressures increase, so does the likelihood of the dies, themselves, fracturing or "zippering" as it is known in the industry.)

The present invention, therefore provides apparatus and process which allow for substantially higher polymer pressures and thus higher throughputs on a per-hole basis relative to normal meltblown die tip construction.

Another major problem in the previous formation of nonwoven fibers and the resultant webs is a phenomenon called "shot". Shot occurs when drawing air is improperly applied to the extruded polymer stream. When this condition occurs, small beads of polymer are formed along with the fibers, thereby giving the formed web a very rough feel. This can be caused by equipment design, improper adjustment of the air to polymer ratio, processing conditions, or a combination of the three. In almost all applications, shot is not desirable. The present invention, however, provides a process and apparatus with increased air flow to and around the extruded polymer, when desired, to decrease shot, and increase fiber formation efficiency or reverse the process when necessary.

As the demands upon nonwoven materials become more complex, it is sometimes desirable to form nonwoven materials which are comprised of intimately entangled fibers of different polymer composition and/or fiber size. The actual generation of materials using more than one polymer and/or fiber typically requires production in a multi-bank layered setup wherein one bank of dies forms fibers of one size or polymer, while another set of dies produces fibers of another size or polymer. The present invention, therefore, provides an apparatus and process which will permit the formation of multi-component nonwoven materials in a more localized and efficient manner.

Another drawback with current meltblowing apparatus and processes are their inability to produce nonwoven materials which are three-dimensional in structure and/or zoned in density in either or both the machine and cross directions. A primary reason for this is the fact that the meltblowing equipment as described in the above references is planar in design and must operate on a continuous basis due to the heating requirements of the polymer and the problem with die holes plugging with stagnant polymer. Consequently, such equipment cannot be cycled on and off to create nonwoven materials having varying densities and other attributes.
The present invention, therefore, provides an apparatus and process which allow cyclical release of polymer during the fiber forming process.
With current meltblowing equipment, described in the above references, production runs are made at a specified width which usually corresponds to the width of the bank of meltblown die tips or openings. To change widths, holes must be plugged or the system shut down to refit the line with smaller or larger banks of die tips. The present invention, therefore provides an apparatus and process which allow on-line variations in production widths of the nonwoven material. Lastly, current meltblowing equipment often becomes clogged when the small die openings become filled with solidified polymer. Usually, there is very little that can be done to unclog the holes while the machinery is running. While a few clogged holes will usually not affect production quality, once enough of the holes become clogged, the die tip must be taken off-line and cleaned - -a costly and time-consuming process.

The present invention therefore also provides a process and apparatus which is self-cleaning. These and other features and advantages of the present invention will become more apparent upon a further review of the following specification and drawings.

In accordance with the present invention there is provided a process for forming fibers from a fiber forming resin comprising the steps of forming a flow of resin from a die housing having at least one resin outlet orifice, said flow extending along a first axis, wherein the resin outlet orifice is recessed within the die housing, and fiberizing said resin to form fibers by flowing a primary fiberization fluid in completely surrounding contact with said flow of resin, said primary fiberization fluid being spiraled about the polymer source as it is extruded through the die tip, and said primary fiberization fluid contacting said flow of resin at a primary fluid flow angle of between about 15 and 60 degrees, said angle being measured as an interior angle between the intersection of the first axis of said flow of resin and a line tangent to the flow of said primary fiberization fluid.

In another aspect of the present invention there is provided an apparatus (10) for forming fibers (22) from a fiber forming resin comprising a die housing (29) including a resin chamber for receiving a supply of molten fiber forming resin, said chamber having a resin outlet orifice (41) in fluid communication therewith for emitting said molten resin in the form of a flow, said flow defining a first axis (61), primary fiberization means (43) completely surrounding said resin outlet orifice (41) for drawing said resin into fibers (22), characterized in that the resin outlet orifice is recessed within the die housing, and in that said primary fiberization fluid is spiraled about the polymer source as it is extruded through the die tip.

An apparatus of the type for forming a nonwoven web from a fiber forming thermoplastic polymer resin, may include reservoir means for supplying a quantity of melted fiber forming thermoplastic polymer resin and pump means for pumping the resin from the reservoir means to a fiber forming die. Die means forms a discrete flow of resin which may be pumped from the reservoir means. The die means includes fiberization means for forming fibers from the flow of resin utilizing first fluid passage means for forming a stream of fluid, such as air, which may contact and substantially surrounds the formed flow of resin for a predetermined distance within the die means. The fiberization means may further include a second fluid passage means for further contacting and attenuating the formed fibers. Receiver means may be spaced at an adjustable predetermined distance from the die means and may collect the fibers formed from the fluid passage means, thereby forming the nonwoven web. A hydraulically actuated stem within the die means may provides an on/off control for selectively stopping flow of the fiber forming resin. The stem may be further used to dislodge resinous debris from the die means.

Other advantages of the present invention will be readily appreciated as the same becomes better understood by reference to the following detailed description when considered in connection with the accompanying drawings wherein:
Figure 1 is a schematic illustration of an apparatus constructed in accordance with the present invention;
Figure 2 is a cross-sectional view of the die constructed in accordance with the present invention;
Figure 3 is a top plan view of a die plate;
Figure 4 is a cross-sectional view taken substantially along lines 4-4 of Figure 3;
Figure 5 is an enlarged fragmentary cross-sectional' view of the nozzle within the die assembly;
Figure 6 is a side view of a nozzle constructed in accordance with the present invention;
Figure 7 is a plan view taken substantially along lines 7-7 of Figure 6;
Figure 8 is a side view of another nozzle constructed in accordance with the present invention;
Figure 9 is an end view of the nozzle shown in Figure 8;
Figure 10 is another side view of the nozzle of Figure 6 showing the flute spiral angle G'.
Figure 11 is a perspective view of the nozzle of Figure 6 showing the flute attack angle H';
Figure 12 is a side view of yet another embodiment of a nozzle constructed in accordance with the present invention.
Figure 13 is a plan view taken substantially along lines 13-13 of Figure 12.

An apparatus of the type for forming a nonwoven web from a fiber forming thermoplastic polymer resin is shown schematically at 10 in Figure 1. Generally, the apparatus includes a reservoir 12 for supplying a quantity of melted fiber forming thermoplastic polymer resin. Such resins are well known in the art. Examples of such resins which can be used in the practice of the present invention include but are not limited to polypropylene, polyethylene, polyester, polyetherester copolymer, polyurethane, polyether-amide copolymer, and styrene-ethylene, butylene copolymer. Furthermore, the properties of such polymers and copolymers may be further enhanced by the addition of various flow modifiers and other additives well known to those skilled in the art.

Many of these polymers are difficult if not impossible to run at high speed throughputs on existing equipment, such as meltblown equipment, due to the high viscosities of the polymers which can cause zippering of the die at increased pressures. Examples of such polymers include PET polyesters, styrene-ethylene, butylene copolymers, and polyetherester copolymers. As demonstrated by the examples below, these polymers can be extruded using the process and apparatus of the present invention.

The reservoir 12 generally includes means for melting the polymer resin and maintaining the resin in the molten state. Typical resins melt at temperatures in the range of 149 to 260 degrees C. Therefore, the reservoir must be able to maintain resin temperatures to at least within this range. A pump 14 pumps the molten resin from the reservoir 12 to one or more fiber forming dies generally indicated at 16. The apparatus 10 includes a source of pressurized air 18 for operating an on/off control means discussed below and a source of fiberization fluid 20 to fiberize the molten resin as discussed below. Note that a single die 16 or a multiple die assembly, as in Figures 3 and 4, may be used to form fibers and nonwoven materials according to the present invention.

The fibers 22 emanating from the die 16 are collected on a receiver assembly such as a continuous wire forming belt 24 in the form of a web 26. The receiver assembly can include means 27 for producing a vacuum beneath the receiving portion of the belt 24 to effectively hold the web 26 to the belt surface and affect the density of the resultant nonwoven web 26. The receiving surface of the belt 24 is spaced at a predetermined distance A' from the die 16. The formed web 26 may be collected on a wind-up roller 28. Alternatively, the web 26 may be further processed downstream from the formation process. Generally, the forming distance A' is between about 7 and 100 centimeters.

Referring to Figure 2, the fiber forming die 16 in its simplest terms can be viewed as having a main housing 29 for receiving a die assembly including a resin nozzle 31 which is fitted within an air forming chamber 33 and capped with an air plate 35. The air plate 35 may include a plurality of openings for being seated over a plurality of nozzles. Figures 3 and 4 show four assemblies 36 in alignment. Alternatively, the assemblies may be aligned in a plurality of rows or staggered to increase the number of openings per unit width. The resin nozzle 31 is in turn fitted with a retractable plunger assembly 37 (a part of the on/off control means) which will permit interruption of the resin flow and cleaning of the nozzle orifice. The die 16 is adapted to receive supplies of both air and molten resin. The air is separately used to operate the retractable plunger assembly 37 and to draw and attenuate the molten resin into fibers as will be explained in more detail below.

Referring to Figure 2, in tracing the flow of the molten resin from entry to exit of the die 16, the molten resin first enters the main housing 29 of the die 16, through the resin inlet port 38 which leads to the interior of the nozzle 31 located within the die 16. The nozzle 31 contains a resin chamber or main flow body 39 which houses and surrounds the hydraulically actuated plunger assembly 37. Consequently, the resin inlet port 38 and main flow body 39 are in fluid communication with one another. As the molten resin enters the main flow body 39 it fills and pressurizes the chamber. The molten resin is then released from the chamber through a resin fluid capillary 40 to form fibers via a resin outlet orifice 41 located within the air plate assembly 35. Initially, the plunger assembly 37 is seated against the base of the resin outlet orifice 41 thereby preventing release of the molten resin. When the plunger 37 is retracted and therefore unseated from the resin outlet orifice 41, the resin is then permitted to escape from the main flow body 39 and thus begin the formation of the fibers 22.

To fiberize and attenuate the resin exiting the resin outlet orifice 41 fiberization/attenuation air or other fluid is used to being spiraled about the polymer source and draw the resin into fibers 22. Consequently, the die means 16 is equipped with primary and, if desired, secondary fiberization means for drawing and attenuating the fibers 22.

Air or another fluid fiberization source enters the die 16 through a fluid inlet port 42. As can be seen from Figure 2, the fluid inlet port 42 is in fluid communication with the air forming chamber 33 which is formed by the space between the interior of the main die housing 29/air plate 35 of the die 16 and the exterior of the nozzle 31. The air forming chamber 33 surrounds at least the lower portion of the nozzle 31 and extends into the air plate assembly 35 where it terminates in an annular fluid outlet port 43. The fluid outlet port 43 typically has a diameter ranging from 3.0 to 5.0 millimeters. It is this fluid outlet port 43 which forms the primary means for attenuating and fiberizing the fibers 22. As the fluid outlet port 43 is reduced in diameter the fiberization/attenuation air is increased in velocity causing the fibers 22 to be attenuated more severely.

To further attenuate and fiberize the molten fibers 22, a secondary fiberization means may also be used. Referring to Figures 2 and 3, the air plate assembly 35 may be fitted with secondary fluid outlet ports 44 spaced radially and axially outward from the first or primary fluid outlet port 43 to create a plurality of secondary fluid streams which impinge upon and further fiberize the molten resin into fibers. These secondary fluid outlet ports 44 are in fluid communication with the air supply 20 via fluid channels 45 which connect the secondary fluid outlet ports 44 with the air forming chamber 33. Alternatively, and not shown, the secondary fluid outlet ports 44 may be connected to an independent pressurized fluid source so the type and/or pressure of the fluid emanating therefrom may be controlled independently of the primary fiberization fluid. Important to proper fiber and web formation is the balance between the formation of the fibers and their subsequent attenuation. Thus the design and interaction between the nozzle 31 with its resin outlet 41 and the primary and secondary fiberization fluid streams will be set forth in yet further detail.

As shown in more detail in Figure 5 and in conjunction with Figure 2, the resin outlet orifice 41 and annular fluid outlet port 43 come together directly above an annular Wall 46 located in the air plate 35 of the die 16. The height of the annular wall 46 is defined by the distance B' between lines 48 and 49. This distance B' is currently limited by machining capabilities; however, the height B' of annular wall 46 is preferably less than 0.5 millimeters. If this height becomes excessively large, molten resin emanating from the resin outlet 41 will collect on the annular wall 46, thus causing large droplets of molten resin to be conveyed onto the formed web 26. These large droplets are called "shot" and may or may not be desirable depending upon the end use of the fibers/nonwoven web.

Because the resin outlet orifice 41 and fluid outlet port 43 come together directly above the annular wall 46, the nozzle 31 and thus the resin outlet orifice 41 can be changed relative to the air plate 35 to vary the amount of recess within the die 16. This distance C' is measured between the end of the resin outlet orifice 41 (line 50) and the bottom of the annular wall 46 (line 48). By adjusting this distance C', the effects of the air flowing from fluid outlet port 43 can be varied to fine tune the fiberization of the molten resin. Preferably, the recess distance C' is greater than O and up to 5 millimeters, although the distance depends upon air flow requirements, polymer viscosity and various other factors which in combination result in the effective control and fiberization of the molten resin. At 0.0 millimeters or no recess the end of the nozzle, i.e., the resin outlet orifice 41, and the' fluid outlet port 43 would lie substantially in the same plane defined by the exterior surface of the air plate portion 35 of the die housing 29. This same plane would also include line 48 shown in Figure 5. Generally, as the distance C' is decreased, the air emanating from the fluid outlet port 43 is at a higher velocity causing the resin emanating from the resin outlet orifice 41 to be attenuated more severely. Conversely, as the distance C' is increased, the air emanating from the fluid outlet port 43 is at a lower velocity causing the resin emanating from the resin outlet orifice 41 to be attenuated less severely. Also note that in certain instances the nozzle 31 could extend beyond the plane defined by the exterior surface of the die housing 29.

Referring to Figures 2 and 5, air is fed to the fluid outlet port 43 via the inlet port 42 in the side of the main housing 29 in die 16. The inlet port 42 directs the air into the air forming chamber 33 which surrounds the nozzle 31 and which is in communication with the fluid outlet port 43 in the air plate 35. The air forming chamber 33 has a cavity surface generally shown at 56. The cavity surface 56 has a substantially cylindrical portion 58 having a substantially annular shape when viewed in cross section and a second frustoconical portion 60 located within the air plate 35. Surface 60 is inclined at what is termed the primary fluid flow angle defined by angle D' in Figures 4 and 5. This is the angle at which the primary fiberization fluid is directed at the flow of molten resin which is traveling along first axis 61. The primary fluid flow angle D' is the angle between the vertical or first axis 61 of the nozzle 31 and a line 51 tangent to the surface of the frustoconical portion 60. Generally, the primary fluid flow angle D' should be between about 15 and 60 degrees. Also note that this first axis 61 defines the initial flow path of the molten resin as it exits the resin outlet orifice 41.

Referring to Figures 2 through 5, the air plate' assembly 35 may be equipped with secondary fluid outlet ports 44 spaced radially and axially outward from the first or primary fluid outlet port 43 to create a plurality of secondary fluid streams which impinge upon and further fiberize the molten resin into fibers. These secondary fluid outlet ports 44 are in fluid communication with the air supply 20 via fluid channels 45 which connect the secondary fluid outlet ports 44 with the air forming chamber 33. Alternatively, and not shown, the secondary fluid outlet ports 44 may be connected to an independent fluid source so the type and/or pressure of the fluid emanating therefrom may be controlled independently of the primary fiberization source. Note too that the secondary fluid outlet ports 44 may have round or other shaped cross-sections of varying dimensions to produce different fiber forming effects.

The secondary fluid outlet ports 44 are angled radially inward towards the longitudinal axis 61 of the nozzle 31 so that the secondary fiberization fluid impinges upon the preliminarily formed fibers 22 at a predetermined angle. This angle is called the secondary fluid flow angle E' and is measured as the interior angle between the first axis of the resin flow (also the longitudinal axis 61 of nozzle 31) and a line 52 tangent to any one of the fluid streams emanating from the secondary fluid outlet ports 44. See Figure 5. This angle E' may be varied between 1 and 45 degrees.

The concave bottom surface 62 of the air plate 35 in combination with the primary and secondary fiberization fluid flows provides a confined fiberization area wherein the primary fiberization fluid through outlet port 43 contacts and substantially surrounds the flow of resin from resin outlet orifice 41. Next, the secondary fiberization fluid impinges upon the preliminarily formed fibers. Upon exiting the die, the fiberization air exiting the primary and secondary fluid outlet ports 43 and 44 behaves as a freely expanding jet. A very high' level of turbulence is created with this type of jet expansion which causes the molten resin stream to be pulled and drawn in random directions, thereby attenuating and fiberizing the molten resin stream to a very high degree. The secondary fiberization streams impinge upon the spread of fibers formed by the primary fiberization fluid flow and at the point of collision of the two flows the fiberization fluid is redirected to produce a non-circular expanding jet as shown by the arrows 63, 64, 65 and 66 in Figure 5. This type of turbulent fiberization process is similar to the meltblowing process which is common within the industry. In contrast, however, the process and apparatus of the present invention allows throughputs on a per-hole basis which are as much as 50 times those compared with current meltblown equipment and techniques. With continuous filament fiberization processes, such as spunbonding, the fiberization air is controlled in the laminar region. This causes the molten resin to be attenuated in a controlled environment. The advantages of the turbulent fiberization process is that a higher degree of attenuation can be achieved than is possible through the laminar, continuous filament process. This higher degree of attenuation can result in the formation of smaller size fibers.

Besides variations in the primary and secondary fiberization fluid flow about the fibers, variations can also be made in the nozzle 31 to affect fiber formation. As shown in more detail in Figures 6 and 7, a first embodiment of the nozzle 31 includes a first axial portion 68 having a first predetermined radial extent and with an axial end portion 70 including a land surface 72, the land surface 72 including the resin outlet orifice 41. The axial end portion 70 has a second predetermined radial extent which is less than the first radial extent of the first axial portion 68. The nozzle portion 31 further includes a tapered axial portion 74 extending between the first axial portion 68 and the axial end portion 70. The angle of the tapered axial portion 74 is defined as the interior angle F' between the longitudinal axis 61 of the nozzle 31 and a line 73 tangent to the surface of the frustoconical portion 74. Generally, this frustoconical angle F' is between about 15 and 60 degrees. In addition, the nozzle 31 may include a threaded end portion 75 for connecting the nozzle 31 into the main housing 29 of the die 16.

The nozzle 31 may include further means for directing the flow of the fluid thereabout. This fluid flow directing means may comprise a plurality of flutes 76 on the outer surface of the nozzle 31. The flutes 76 may extend over the tapered axial portion 74, the axial end portion 70, and into the land surface 72.

In a second embodiment of the nozzle portion of the present invention shown in Figures 8 and 9 wherein like structures are shown by primed numbers, the nozzle 31' does not include an axial end portion 70. Rather, the land surface 72' is directly adjacent the distal edge of the tapered axial portion 74'. As shown in both the embodiments of Figures 7 and 9, the flutes 76, 76' extend into the land surfaces 72, 72'.

The fiberization air source 20 provides a primary air flow supply entering into the die through the fluid inlet 42 shown in Figure 2. The inner cavity 33 provides a balancing channel for distributing the incoming air about the nozzle 31. The air balances around the nozzle 31 and is then directed towards the fluid outlet port 43 of the air flow channel defined within the cavity 33 due to the air pressure utilized in the system. This primary air flows over the flutes 76, 76' that have been cut into the outside diameter of the nozzle on compound angles thereby causing the fiberization air to spiral about and attenuate the newly-formed fibers 22.

The flute spiral angle G' around the nozzle tip is the interior angle measured between the first axis 61 of the nozzle 31 and a line 78 parallel to the longitudinal axis of one of the flutes 76, shown as angle G' in Figure 10. The flute spiral angle G' should generally be between about 20 and 45 degrees. This spiral angle determines the rotational and centrifugal force of the fluid flow acting on the molten resin stream emitted from the resin outlet orifice 41.

The flute attack angle H' determines how quickly the air contacts the resin stream. This angle is the angle measured between the longitudinal axis 61 of the nozzle 31 and a line 79 parallel to the interior surface 83 of one of the flutes 76. See Figure 11. The attack angle H' in conjunction with the angle of the frustoconical portion 60 of the air forming chamber 33 determines the collision location of the primary air flow as it flows over the flutes 76 and contacts the stream of molten resin which exits the resin outlet orifice 41. The flute attack angle H' should generally range between about 7 and 60 degrees.

In a third embodiment of the nozzle shown in Figures 12 and 13, the nozzle 31 does not include flutes on the tapered axial portion 74 or on the land surface 72. The absence of the flutes in this third embodiment minimizes rotational forces in the air stream. This may be preferred for certain molten polymers which have relatively low melt strength.

It can be seen that there are many surfaces within the die housing 29 which can be varied to modify the flow characteristics and thus the formation of the fibers 22 created by the present apparatus and process. A particularly advantageous feature of the present invention is the interchangeability of the nozzles 31. By removing the air plate 35, the nozzle 31 can be removed and a new nozzle inserted. As a result, changes in resin and fiber formation can be complemented by changes in nozzles.

Additional versatility is added to the present invention by the fact that it is provided with a means for selectively stopping and starting the flow of resin and thus the formation of fibers. In multi-die configurations such as are shown in Figures 3 and 4, it is possible to cycle one, some, or all of the nozzles on and off. As a result, it is possible to interrupt the fiber formation process, thereby creating individual discrete nonwoven webs. In addition, by being able to cycle select nozzles on and off, nonwoven webs can be created with varying basis weight in either or both of the machine-and cross-directions. In in-line processes, such as the formation of personal care products (diapers, sanitary napkins, etc.), it is therefore possible to tailor design specific areas and attributes of the product, as, for example, zoned absorbency. To accomplish this, the apparatus 10 includes on/off control means for selectively stopping and starting resin flow from the resin outlet orifice 41 while simultaneously dislodging resinous debris therefrom.

Referring to Figures 2 and 5, the on/off control means includes a pneumatic fixture generally indicated at 90 which is connected to and therefore forms a part of the main die housing 29. Extending from the pneumatic fixture 90 into the main flow body 39 is a plunger assembly or reciprocating stem 92 having a distal tip 94 located above the resin flow capillary 40. The stem 92 has an unseated condition, as shown in Figures 2 and 5, wherein the tip 94 is retracted into the main flow body 39 and spaced from the capillary 40 and a seated condition (not shown) wherein the stem 92 is reciprocated to seat the tip 94 against the capillary 40. By seating the stem 92, a hydrostatic pressure is created in the capillary 40 which dislodges any debris located therein and restricts flow of molten resin from the resin flow outlet 41.

The pneumatic fixture 90 includes a pneumatic chamber 96, including an upper chamber 96a and a lower chamber 96b, shown in Figure 2. The stem 92 includes an end portion 98 extending into the pneumatic chamber 96. The end portion 98 of the stem 92 has a piston 100 mounted thereon and fitted with seals 102 to contact the walls of chamber 96 to form the upper and lower chambers 96a and 96b, respectively. The chamber 96 includes a pair of hydraulic fluid ports 104, 106 opening into the pneumatic chamber 96 for supplying varying fluid pressure on each side of the piston 100 to reciprocate the piston 100 within the pneumatic chamber 96 thereby reciprocating the stem 92 between the seated (off) and unseated (on) conditions.

The main flow body 39 includes a stem port 108 with the stem 92 extending through the stem port 108. The die 16 includes a high temperature resistant dynamic seal 110 for allowing sliding engagement while perfecting a seal between the stem 92 and the stem port 108 to prevent the passage of molten resin through the port 108. The seal 110 can be U-shaped in cross-section so as to expand into the space between the stem 92 and the wall of the port 108 upon pressure applied by the incoming polymer resin. Thus, the seal 110 provides a separation between the molten material and the outside environment under molten material pressure conditions. The seal mechanism should provide a positive seal at temperatures up to 350 degrees C.

Operation of the on/off mechanism involves selectively pressurizing either the upper chamber 96a or the lower chamber 96b. To turn the mechanism on and start the flow of molten resin from resin outlet orifice 41, the pressure from upper chamber 96a is relieved through fluid port 104 and pressurized air is fed into lower chamber 96b via fluid port 106. As a result of the pressure imbalance on either side of the piston 100, the piston 100 moves further into the upper chamber 96a unseating the tip 94 of the stem 92 from the capillary 40 and thereby allowing the release of the molten resin from the main flow body 39 through resin outlet orifice 41. To turn off the mechanism and interrupt the flow of molten resin the above procedure is reversed. Namely, the pressure from the' lower chamber 96b is decreased and the pressure in the upper chamber 96a is increased, again causing a pressure imbalance which forces the tip 94 of stem 92 to seat against the capillary 40 and cut off the flow of molten resin. Additionally, this action will create a sufficient hydrostatic pressure within capillary 40 to dislodge any debris located therein. Alternatively, it should be appreciated that the pneumatic fixture 90 may be modified by, as an example, adding a mechanical spring (not shown) within one of the chambers 96a or 96b to further act upon the piston 100 to maintain the stem 92 in either a seated or unseated condition absent the use of air pressure in the opposite chamber. Thus, the present invention can be utilized under varying conditions to provide a very useful range of throughputs, significantly higher than meltblowing processes.

A process for forming the nonwoven web 16, generally includs the steps of supplying a quantity of melted fiber-forming thermoplastic resin, pumping the resin to the fiber-forming die 16, forming a discrete flow of resin to flow from the die 16, flowing a stream of fiberization fluid, such as air, in contact and substantially surrounding the formed flow or resin, and collecting the formed fibers at a predetermined distance A' from the die 16. More specifically, the flow of fiberization fluid is contained completely about the resin for a predetermined distance, the distance being called the die recess distance C' which is the distance between lines 48 and 50 in Figure 5. This distance is varied by recessing the outlet orifice from the primary air opening 43.

The method further includes the step of balancing the fluid flow from the fluid inlet port 42 about the nozzle 31 within the die 16 in the air forming chamber 33. The flow of fluid is directed about the nozzle 31 by flowing, the fluid over the flutes 76 formed on the exterior of the nozzle 31. The spread of the fibers is directed and further fiberized by forming the secondary fiberization fluid flow including at least two fluid streams impinging on the fibers formed by the substantially surrounding primary air flow and colliding the fluid streams to form a non-circular expanding jet as shown in Figure 5 by arrows 63 through 66. The secondary fiberization fluid, flowing from the two outlet orifices 44 on opposite sides of the surrounding fluid, flows at an angle towards the surrounding fluid flow, defined by angle E' in Figure 5.

The process further includes the step of selectively stopping the flow of resin from the resin outlet orifice 41. To stop the resin flow, the stem 92 is reciprocated so that the distal tip 94 of the stem 92 seats against the surface of the resin outlet capillary 40 to stop the resin flow and unseats the distal tip 94 from the resin outlet capillary 40 to unstop the resin flow. The seating of the distal tip 94 creates a hydrostatic pressure in the capillary 40 to dislodge debris from the capillary 40 and the resin outlet orifice 41. The stem 92 reciprocates by pneumatic actuation of the piston 100 connected to the stem 92 disposed within the pneumatic chamber 96 to seat and unseat the distal tip 94. The stem 92 can be reciprocated with short or long strokes.

In operation, the resin outlet orifice 41 has a preferred diameter of between 0.5 and 1.0 millimeters, although trials have shown effective fiberization utilizing a polymer orifice diameter of up to 3 millimeters. The nozzle recess C' has been varied between greater than 0 and 5 millimeters with resulting effective fiberization. The nozzle temperature has been varied between 138 and 330 degrees C. Tests have shown an effective air flow of 56 to 1558 standard liters per minute per nozzle with resulting effective fiberization. Nozzle air pressure has been varied between 6.9 and 172 kPa with some trials utilizing pressures as high as 317 kPa. Fiberization air temperatures have been varied between 137 and 343 degrees C depending on the polymer utilized. A forming distance A' between the nozzle tip and the landing area of the receiving belt has been varied between 15 and 64 centimeters although some trials have been successful utilizing a distance as low as 7.5 centimeters or as high as 102 centimeters. Polymer throughput has been varied between 0.76 and 38 grams per minute per nozzle although other trials have achieved throughputs up to 151 grams per minute per nozzle and as low as 0.1 grams per minute per nozzle. Polymers which can be fiberized with the present invention include, but are not limited to, polypropylene, polyethylene, polybutylene, PET polyester, PETG copolyester, PBT polyester, ethylene vinyl acetate copolymer, polyurethane, polyetherester copolymers, and styrene/ethylene-butylene copolymers.

To demonstrate the functional attributes and properties of the apparatus and products produced by the present invention, a series of experiments, as presented below, were run using an apparatus of the type shown schematically in Figure 1 and including a general die tip assembly such as is shown in Figure 2. In all the examples, structurally both the nozzle tip geometry and the air plate geometry can be varied to change the characteristics of the resultant fiber formation. In addition, both the nozzle recess distance and the forming distance between the die and the receiver can be varied to affect the fiber formation and the attributes of the resultant nonwoven web. Depending upon the particular polymer used, other factors can be varied to affect fiber formation including the melt temperature of the polymer, the polymer throughput rate in grams per hole (nozzle) per minute, air flow in standard liters per minute per nozzle, and lastly, air temperature of the forming air. In most cases, the resin was extruded through a four-nozzle head assembly. However, in Examples VIII, IX, XIII and XIV, a single-nozzle assembly was used; in Example IV an eight nozzle assembly was used, and in Example XII an eighteen nozzle assembly was used. All data are given on a per hole (nozzle) basis.

### EXAMPLE I

A PET polyester manufactured by Eastman Chemical Products, Inc. and designated No. 9028 was extruded at a melt temperature of 287 degrees C at a throughput of 3.1 grams per hole per minute resulting in a melt pressure of 455 kPa. The fiberization fluid was air at a flow rate of 177 standard liters per minute per nozzle with an air temperature of 293 degrees C. The nozzles located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 45 degrees. The nozzle recess distance was 2 millimeters and the forming distance between the die and the receiver was 38.10 centimeters. Under the above conditions, the average fiber diameter was 15.5 µm the web formed from the extruded fibers had a density of approximately 0.061 grams per cubic centimeter and the average shot size using an optical microscope was 0.015 square millimeters.

### EXAMPLE II

A PETG copolyester manufactured by Eastman Chemical Products, Inc. and designated Kodar 6763 was extruded at a melt temperature of 287 degrees C at a throughput of 7.4 grams per hole per minute, resulting in a melt pressure of 896 kPa. The fiberization fluid was air at a flow rate of 127 standard liters per minute per nozzle with an air temperature of 283 degrees C. The nozzles located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 2.0 millimeter diameter with a 180 degree separation. The secondary fluid flow angle was 45 degrees. The nozzle recess distance was 2 millimeters and the forming distance between the die and the receiver was 58 centimeters. Under the above conditions, the average fiber diameter was 24.9 µm the web formed from the extruded fibers had a density of approximately 0.050 grams per cubic centimeter and the average shot size using an optical microscope was 0.0076 square millimeters.

### EXAMPLE III

Polyurethane manufactured by B. F. Goodrich and designated Estane 5740x732 was extruded at a melt temperature of 216 degrees C at a throughput of 6.6 grams per hole per minute resulting in a melt pressure of 827 kPa. The fiberization fluid was air at a flow rate of 184 standard liters per minute per nozzle with an air temperature of 232 degrees C. The nozzles located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 25 degrees. The nozzle recess distance was 2 millimeters and the forming distance between the die and the receiver was 15 centimeters. Under the above conditions, the average fiber diameter was 24 µm the web formed from the extruded fibers had a density of approximately 0.150 gm/cm³ and the average shot size using an optical microscope was 0.0098 square millimeters.

### EXAMPLE IV

A styrene-ethylene-butylene-styrene copolymer manufactured by The Shell Chemical Company and designated Kraton G-2740X was extruded at a melt temperature of 238 degrees C at a throughput of 3.7 grams per hole per minute resulting in a melt pressure of 586 kPa. The fiberization fluid was air at a flow rate of 120 standard liters per minute per nozzle with an air temperature of 263 degrees C. The nozzles located within the die housing had a first axial portion diameter of 12 millimeters, a cylindrical end portion diameter of 4 millimeters, a resin outlet orifice diameter of 1 millimeter with the angle of the frustoconical section being 45 degrees. The nozzles included six flutes having a flute spiral angle of 20 degrees and a flute attack angle of 45 degrees. Air flow geometry included a primary air opening diameter of 4 millimeters, a primary fluid flow angle of 45 degrees and three secondary air orifices on each side of the primary air openings, all having a 1.5 millimeter diameter. The secondary fluid flow angles were each 45 degrees. The nozzle recess distance was 2 millimeters and the forming distance between the die and the receiver was 23 centimeters. Under the above conditions, the average fiber diameter was 86 µm, the web formed from the extruded fibers had a density of approximately 0.161 gm/cm³ and the average shot size using an optical microscope was 0.025 square millimeters.

### EXAMPLE V

A polymer containing by weight 83% Dow Chemical Aspun 6814 polyethylene, 12% Allied Chemical AC-9 polyethylene, 4% blue polyethylene coloring and 1% wetting agent was extruded at a melt temperature of 232 degrees C at a throughput of 18.9 grams per hole per minute using a melt pressure of 2758 kPa. The fiberization fluid was air at a flow rate of 348 standard liters per minute per nozzle with an air temperature of 210 degrees C. The nozzles located within the die housing had a first axial portion diameter of 12 millimeters, a cylindrical end portion diameter of 5 millimeters, a polymer exit orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices with 180 degrees separation, both having a 2 millimeter diameter. The secondary fluid flow angle was 45 degrees. The nozzle recess distance was 4 millimeters and the forming distance between the die and the receiver was 54 centimeters. Under the above conditions, the average fiber diameter was 21 µm, the web formed from the extruded fibers had a density of approximately 0.072 gm/cm³ and the average shot size using an optical microscope was 0.24 square millimeters.

### EXAMPLE VI

A blend of 93.5% Himont Profax PF-015 polypropylene, 4.0% Standridge Color Corp. 5834 blue polypropylene color concentrate and 2.5% wetting agent was extruded at a melt temperature of 235 degrees C at a throughput of 18.9 grams per hole per minute resulting in a melt pressure of 1172 kPa. The fiberization fluid was air at a flow rate of 266 standard liters per minute per nozzle with an air temperature of 235 degrees C. The nozzles located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 4 millimeters, a primary fluid flow angle of 45 degrees and two 1.5 millimeter diameter secondary air orifices on each side of the primary air openings. The secondary fluid flow angle was 45 degrees. The nozzle recess distance was 2 millimeters and the forming distance between the die and the receiver was 48 centimeters. Under the above conditions, the average fiber diameter was 21 µm, the web formed from the extruded fibers had a density of approximately .080 gm/cm³ and the average shot size using an optical microscope was 0.11 square millimeters.

### EXAMPLE VII

Profax PF-015 polypropylene was extruded at a melt temperature of 260 degrees C at a throughput of 2.8 grams per hole per minute resulting in a melt pressure of 103 kPa. The fiberization fluid was air at a flow rate of 545 standard liters per minute per nozzle with an air temperature of 260 degrees C. The nozzles located within the die housing had a first axial portion diameter of 12 millimeters, a cylindrical end portion diameter of 1.25 millimeters and a resin outlet orifice diameter of 1 millimeter with the angle of the frustoconical section being 30 degrees. The nozzles had no flutes. Air flow geometry included a primary air opening diameter of 3 millimeters, a primary fluid flow angle of 30 degrees and three secondary air orifices on each side of the air plate, all having a 1.5 millimeter diameter. The secondary fluid flow angle was 45 degrees. The nozzle recess distance was 0.5 millimeters and the forming distance between the die and the receiver was 48 centimeters. Under the above conditions, the average fiber diameter was 2.3 µm the web formed from the extruded fibers had a density of approximately 0.069 gm/cm³ and the average shot size using an optical microscope was 0.034 square millimeters.

### EXAMPLE VIII

Himont Profax PF-015 polypropylene was extruded at a melt temperature of 260 degrees C at a throughput of 148 grams per hole per minute resulting in a melt pressure of 1710 kPa. The fiberization fluid was air at a flow rate of 1558 standard liters per minute per nozzle with an air temperature of 260 degrees C. The nozzle located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzle included six flutes having a flute spiral angle of 20 degrees and a flute attack angle of 7 degrees. Air flow geometry included a primary air opening diameter of 5 millimeters, a primary fluid' flow angle of 45 degrees and two secondary air orifices both having a 1.5 millimeter diameter with a 180 degree separation. The secondary fluid flow angle was 45 degrees. The nozzle recess distance was 2 millimeters and the forming distance between the die and the receiver was 38 centimeters. Under the above conditions, the average fiber diameter was 30 µm the web formed from the extruded fibers had a density of approximately 0.069 gm/cm³ and the average shot size using an optical microscope was 0.30 square millimeters.

### EXAMPLE IX

Himont Profax PF-015 polypropylene was extruded at a melt temperature of 260 degrees C at a throughput of 37 grams per hole per minute using a melt pressure of 690 kPa. The fiberization fluid was air at a flow rate of 651 standard liters per minute per nozzle with an air temperature of 260 degrees C. The nozzles located within the die housing had a first axial portion diameter of 12 millimeters, a cylindrical end portion diameter of 5 millimeters, a polymer exit orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 45 degrees. The nozzle recess distance was 2 millimeters and the forming distance between the die and the receiver was 38 centimeters. Under the above conditions, the average fiber diameter was 3.1 µm the web formed from the extruded fibers had a density of approximately 0.049 gm/cm³ and the average shot size using an optical microscope was 0.078 square millimeters.

### EXAMPLE X

Arnitel EM-450 polyetherester copolymer manufactured by Akzo was extruded at a melt temperature of 266 degrees C at a throughput of 2.95 grams per hole per minute resulting in a melt pressure of 869 kPa. The fiberization fluid was air at a flow rate of 404 standard liters per minute per nozzle with an air temperature of 264 degrees C. The nozzles located within the die housing had a first axial portion diameter of 12 millimeters, a cylindrical end portion diameter of 5 millimeters, a resin outlet orifice diameter of 1 millimeter with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 25 degrees. The nozzle recess distance was 2 millimeters and the forming distance between the die and the receiver was 24 centimeters. Under the above conditions, the average fiber diameter was 12 µm, the web formed from the extruded fibers had a density of approximately 0.104 gm/cm³ and the average shot size using an optical microscope was 0.058 square millimeters.

### EXAMPLE XI

Himont Profax PF-015 polypropylene was extruded at a melt temperature of 260 degrees C at a throughput of 23 grams per hole per minute resulting in a melt pressure of 1931 kPa. The drawing air was at an air flow rate of 375 standard liters per minute per nozzle with an air temperature of 274 degrees C. The nozzles located within the die housing had a first axial portion diameter of 12 millimeters, a cylindrical end portion diameter of 4 millimeters, a resin outlet orifice diameter of 0.5 millimeters with the angle of the frustoconical section being 45 degrees. The nozzles included six flutes having a flute spiral angle of 20 degrees and a flute attack angle of 7 degrees. Air flow geometry included a primary air opening diameter of 5 millimeters, a primary fluid flow angle of 45 degrees and two secondary air orifices each having a 2 millimeters diameter with a 180 degree separation. The secondary fluid flow angle was 45 degrees. The nozzle recess distance was 2 millimeters and the forming distance between the die and the receiver was 13 centimeters. Under the above conditions, the average fiber diameter was 5.7 µm the web formed from the extruded fibers had a density of approximately 0.035 gm/cm³ and the average shot size using an optical microscope was 0.079 square millimeters.

### EXAMPLE XII

Profax PF-015 polypropylene was extruded at a melt temperature of 260 degrees C at a throughput of 0.34 grams per hole per minute resulting in a melt pressure of 69 kPa. The fiberization fluid was air at a flow rate of 136 standard liters per minute per nozzle with an air temperature of 304 degrees C. The nozzles located within the die housing had a first axial portion diameter of 12 millimeters, a cylindrical end portion diameter of 1.25 millimeters, a resin outlet orifice diameter of 1 millimeter with the angle of the frustoconical section being 30 degrees. The nozzles had no flutes. Air flow geometry included a primary air opening diameter of 4' millimeters, a primary fluid flow angle of 45 degrees and three secondary air orifices on each side of each resin outlet orifice, all having a 1.5 millimeter diameter. The secondary fluid flow angle was 45 degrees. The nozzle recess distance was 2 millimeters and the forming distance between the die and the receiver was 39 centimeters. Under the above conditions, the average fiber diameter was less than 2.0 , the web formed from the extruded fibers had a density of approximately 0.039 gm/cm³ and the average shot size using an optical microscope was 0.020 square millimeters.

### EXAMPLE XIII

Himont Profax PF-015 polypropylene was extruded at a melt temperature of 260 degrees C at a throughput of 38.4 grams per hole per minute resulting in a melt pressure of 462 kPa. The fiberization fluid was air at a flow rate of 1104 standard liters per minute per nozzle with an air temperature of 260 degrees C. The nozzle located within the die housing had a first axial portion diameter of 12 millimeters, a cylindrical end portion diameter of 5 millimeters, a resin outlet orifice diameter of 2 millimeters with the angle of the frustoconical section being 45 degrees. The nozzle included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 45 degrees. The nozzle recess distance was 2 millimeters and the forming distance between the die and the receiver was 38 centimeters. Under the above conditions, the average fiber diameter was 3.3 µm the web formed from the extruded fibers had a density of approximately 0.095 gm/cm³ and the average shot size using an optical microscope was' 0.14 square millimeters.

### EXAMPLE XIV

Himont Profax PF-015 polypropylene was extruded at a melt temperature of 260 degrees C at a throughput of 38.3 grams per hole per minute resulting in a melt pressure of 283 kPa. The fiberization fluid was air at a flow rate of 651 standard liters per minute per nozzle with an air temperature of 260 degrees C. The nozzle located within the die housing had a first axial portion diameter of 12 millimeters, a cylindrical end portion diameter of 5 millimeters, a resin outlet orifice diameter of 3 millimeters with the angle of the frustoconical section being 45 degrees. The nozzle included six flutes having a flute spiral angle of 20 degrees and a flute attack angle of 7 degrees. Air flow geometry included a primary air opening diameter of 5 millimeters, a primary fluid flow angle of 45 degrees and two secondary air orifices both having a 1.5 millimeter diameter with a 180 degree separation. The secondary fluid flow angle was 45 degrees. The nozzle recess distance was 2 millimeters and the forming distance between the die and the receiver was 38 centimeters. Under the above conditions, the average fiber diameter was 3.1 the web formed from the extruded fibers had a density of approximately 0.065 gm/cm³ and the average shot size using an optical microscope was 0.075 square millimeters.

From the foregoing examples, it can be seen that the process and apparatus of the present invention permit the formation of fibers and resultant nonwoven webs from a wide variety of polymers under various conditions. Typical meltblown equipment under the very best of conditions can only process standard polymers at rates of no more than 3 grams per hole per minute. 'With certain polymers, even these throughputs are not possible due to the danger of the meltblown dies zippering. In contrast, the process and the apparatus of the present invention has been shown to be able to process polymers at rates as high as 150 grams per hole per minute. In port, this higher throughput capability is due to the higher melt pressure capability of the nozzle. As spelled out in the working examples, melt pressures up to 2758 kPa can be withstood. Other experiments have shown melt pressures as high as 6900 kPa can be withstood without failure of equipment. This is in contrast to meltblown die tip pressures which are believed to have maximum let pressures of only 2100 kPa. Thus, the present apparatus may be used in single or multiple die configurations which, on a per hole basis, will far exceed current meltblown capabilities. As a result, the apparatus of the present invention may be used in areas where space constraints are critical. In addition, the apparatus may be used to create localized fiber formation thereby permitting the creation of the nonwoven webs having wide variances in their basis weights. Nonwoven webs with variances in their basis weights in excess of 10% have been created by localized increases and/or reductions in fiber formations in either or both of the machine and cross-directions. Consequently, it can be seen that the process and apparatus of the present invention can be applied in a wide variety of applications to enhance current nonwoven forming techniques.

In the following, further advantageous aspects of the invention are described.

According to a first of these aspects a process for forming fibers from a fiber forming resin of claim 1 includes the step of forming a flow of resin from a die housing having at least one resin outlet orifice, the flow extending along a first axis, wherein the resin outlet orifice is recessed within the die housing, and of fiberizing said resin flows to form fibers by flowing a primary fiberization fluid in completely surrounding contact with said flow of resin, said primary fiberization fluid being spiraled about the polymer source as it is extruded through the die tip, and said primary fiberization fluid contacting each said resin flow at a primary fluid flow angle of between about 15 and 60 degrees, said angle being measured as an interior angle between the intersection of the first axis of said flow of resin and a line tangent to the flow of said primary fiberization fluid about said individual flows of resin.

According to a preferred aspect, the process includes the step of further fiberizing said resin flows prior to collecting said fibers by contacting said individual resin flows with a flow of a secondary fiberization fluid including at least two fluid streams which each impinge upon said resin flows at a secondary fluid flow angle of between about 1 and 45 degrees, said angle being measured as an interior angle between the intersection of the first axis of each of said flows of resin and a line tangent to the flow of said secondary fiberization fluid flows about said individual flows of resin.

The process includes the step of angling at least one of said primary fiberization fluid flows such that it spirals about said first axis of said flow of resin.

In still another preferred aspect, the process comprises the step of collecting said fibers in the form of a nonwoven web.

In another aspect, the apparatus according to the invention for intermittently forming fibers from a fiber forming resin comprises: a die housing; including a resin chamber for receiving a supply of molten fiber forming resin, said chamber having a resin outlet orifice in fluid communication therewith for emitting said molten resin in the form of a flow, said flow defining a first axis; primary fiberization means completely surrounding said resin outlet orifice (41) for drawing said flow of molten resin into fibers, the resin outlet orifice is recessed within the die housing, and in that primary fiberization fluid is spiraled about the polymer source as it is extruded through the die tip. Preferably the apparatus comprises on/off control means for selectively interrupting flow of said molten resin from said resin outlet orifice.

In a preferred aspect, a die assembly is located within said housing.

In a preferred aspect, the apparatus with fiberization means includes a primary fiberization fluid which completely surrounds said flow of molten resin.

In another preferred aspect, the apparatus with a die housing includes a fluid outlet port completely surrounding said resin outlet orifice for emitting said primary fiberization fluid.

In yet another preferred aspect, the apparatus with on/off control means includes a plunger within said resin chamber having a closed position wherein said plunger is in contact with said resin outlet orifice to prevent flow of said molten resin from said orifice and an open position wherein said plunger is retracted from said orifice to allow flow of said molten resin from said orifice.

In a further preferred aspect the apparatus with a die housing includes a hydraulic chamber said plunger including an end portion extending into said hydraulic chamber and including a piston mounted thereon, said chamber including hydraulic fluid ports opening into said hydraulic chamber for supplying varying fluid pressure on each side of said piston to reciprocate said piston within said hydraulic chamber to move said plunger between said open and closed positions.

In another preferred aspect according to the invention, the apparatus with fiberization means includes a fluid outlet port in said die housing completely surrounding said flow of resin from said resin outlet orifice and a primary fiberization fluid emanating from said fluid outlet port for fiberizing said resin to form fibers.

In another preferred aspect, the apparatus with fiberization means further includes a secondary fiberization fluid including at least two fluid streams which each impinge upon said flow of resin at a secondary fluid flow angle of between about 1 and 45 degrees, said angle being measured as an interior angle between the intersection of the first axis of said flow of resin and a line tangent to the flow of said fluid stream.

In still another preferred aspect, the apparatus with a die housing further includes a nozzle located therein and at least partially surrounded by a fiberization fluid chamber which terminates in said fluid outlet port, said nozzle including said resin chamber and said resin outlet orifice.

In a further preferred aspect, the nozzle is removably retained within said die housing.

In another preferred aspect, the apparatus with the nozzle has a nozzle exterior surface, said nozzle exterior surface having a plurality of flutes adjacent said resin outlet orifice to direct said primary fiberization fluid.

In a further preferred aspect, the apparatus with the nozzle exterior surface includes a first axial portion having a first predetermined radial extent and an axial end portion having preferably a substantial cylindrical outer surface having a land surface including said resin outlet orifice extending therethrough and having a second predetermined radial extent which is less than said first radial extent, said nozzle including a tapered axial portion extending between said first axial portion and said axial end portion including said plurality of flutes, said flutes extending into said land surface and preferably are situated in the cylindrical outer surface.

In another preferred aspect, the nozzle has a flute attack angle of about 7 to 60 degrees and a flute spiral angle of about 20 to 45 degrees.

In still preferred another aspect, the nozzle has a frustoconical angle of about 15 to 60 degrees.

## Claims

1. A process for forming fibers from a fiber forming resin comprising the steps of:
(a) forming a flow of resin from a die housing having at least one resin outlet orifice, said flow extending along a first axis, wherein the resin outlet orifice is recessed within the die housing, and
(b) fiberizing said resin to form fibers by flowing a primary fiberization fluid in completely surrounding contact with said flow of resin, said primary fiberization fluid being spiraled about the polymer source as it is extruded through the die tip, and said primary fiberization fluid contacting said flow of resin at a primary fluid flow angle of between about 15 and 60 degrees, said angle being measured as an interior angle between the intersection of the first axis of said flow of resin and a line tangent to the flow of said primary fiberization fluid.

2. The process of claim 1 which includes the step of further fiberizing said resin by contacting said resin with a flow of a secondary fiberization fluid including at least two fluid streams which each impinge upon said resin at a secondary fluid flow angle of between about 1 and 45 degrees, said angle being measured as an interior angle between the intersection of the first axis of said flow of resin and a line tangent to the flow of said fluid stream.

3. The process of one of the preceding claims wherein said flow of resin is at a melt pressure of less than or equal to 6900 kPa.

4. The process of one of the preceding claims wherein said flow of resin is at a throughput of about 0.1 to 151 grams per orifice per minute, preferably of about 0.75 to 38.0 grams per orifice per minute.

5. The process of one of the preceding claims, wherein said primary fiberization fluid flows at a rate of about 57 to 1558 standard litres per minute, preferably at a rate of about 57 to 708 standard litres per minute.

6. The process of one of the preceding claims which further includes the step of angling said primary fiberization fluid flow such that it spirals about said first axis of said flow of resin.

7. The process of one of the preceding claims wherein said primary fiberization fluid is at a pressure of between about 6.9 and 317 kPa, preferably of between about 6.9 and 172 kPa.

8. The process of one of the preceding claims wherein said primary fiberization fluid is at a temperature of between about 137°C and 344°C.

9. The process of one of the preceding claims wherein said at least one resin outlet orifice has a diameter of between about 0.25 and 3.0 millimeters, preferably of between about 0.5 and 1.0 millimeters.

10. The process of one of the preceding claims which further includes the step of collecting said fibers in the form of a nonwoven web.

11. The process of claim 10 wherein said collection of said fibers in the form of a nonwoven web takes place at a distance of from about 7.5 to 102 cm, preferably of from about 15 to 64 cm from said resin outlet orifice.

12. A process for forming fibers from a fiber forming resin according to one of the preceding claims, comprising the additional steps of:
(a) pumping a molten fiber forming resin into one or more die assemblies, each of said assemblies having a resin chamber for receiving said molten fiber forming resin and a resin outlet orifice in fluid communication with said chamber for discharging said resin, each said assembly further including a retractable plunger within said resin chamber having a closed position wherein said plunger is in contact with said resin outlet orifice to prevent flow of said resin from said orifice and an open position wherein said plunger is retracted from said resin outlet orifice to allow the flow of said resin from said orifice;
(b) retracting one or more of said plungers from said closed to said open positions to intermittently form flows of resin from said outlet orifices having said plungers in an open position, said flows extending along individual first axes;
(c) interrupting one or more of said flows of resin by selectively cycling said plungers between said open and closed positions.

13. The process of claim 12, wherein said interruption of said flow of resin causes the formation of separate nonwoven webs and/or the formation of a nonwoven web having variations in its basis weight of at least 10 percent.

14. An apparatus (10) for forming fibers (22) from a fiber forming resin comprising:
A die housing (29) including a resin chamber for receiving a supply of molten fiber forming resin, said chamber having a resin outlet orifice (41) in fluid communication therewith for emitting said molten resin in the form of a flow, said flow defining a first axis (61), primary fiberization means (43) completely surrounding said resin outlet orifice (41) for drawing said resin into fibers (22), **characterized in that** the resin outlet orifice is recessed within the die housing, and in that said primary fiberization fluid is spiraled about the polymer source as it is extruded through the die tip.

15. The apparatus of claim 14 wherein said fiberization means includes a fluid outlet port (43) in said die housing completely surrounding said flow of resin from said resin outlet orifice (41) and a primary fiberization fluid emanating from said fluid outlet port (43) for fiberizing said resin to form fibers (22) said primary fiberization fluid contacting said flow of resin at a primary fluid flow angle (D') of between about 15 and 60 degrees, said angle being measured as an interior angle between the intersection of the first axis (61) of said flow of resin and a line tangent (51) to the flow of said primary fiberization fluid.

16. The apparatus of claim 14 and 15 which further includes secondary fiberization means (44) located exteriorly from said primary fiberization means (43) for supplying a secondary fiberization fluid which further fiberizes said resin into fibers (22).

17. The apparatus of claim 16 wherein said secondary fiberization means comprises a secondary fiberization fluid including at least two fluid streams which each impinge upon said flow of resin at a secondary fluid flow angle (E') of between about 1 and 45 degrees, said angle being measured as an interior angle between the intersection of the first axis (61) of said flow of resin and a line tangent (52) to the flow of said fluid stream.

18. The apparatus of claim 17 wherein said at least two fluid streams are symmetrically spaced radically and circumferentially about said first axis (61) exteriorly from said fluid outlet port (41).

19. The apparatus of one of claims 14 to 18, wherein said die housing (29) has an external surface which defines a plane with said resin outlet orifice (41) and said fluid outlet port (43) lying substantially in the same plane defined by said external surface of said die housing.

20. The apparatus of one of claims 14 to 18, wherein said fluid outlet port (43) lies substantially within a plane (48) defined by said external surface of said die housing and said resin outlet orifice (41) is recessed within said die housing a distance (C') not exceeding 5 millimeters as measured from said plane (48).

21. The apparatus of one of claims 14 to 20, wherein said resin outlet orifice (41) has a diameter from about 0.25 to 3.0 millimeters.

22. The apparatus of one of claims 14 to 21 wherein said fluid outlet port (43) has a diameter between about 3 and 5 millimeters.

23. The apparatus of one of claims 14 to 22 wherein said primary fiberization fluid and said secondary fiberization fluid are fed from separate supplies of fluid.

24. The apparatus of one of claims 14 to 23 wherein said die housing (29) further includes a nozzle (31) located therein and at least partially surrounded by a fiberization fluid chamber (33) which terminates in said fluid outlet port (43)said nozzle (31) including said resin chamber and said resin outlet orifice(41).

25. The apparatus of claim 24 wherein said nozzle (31) is removably retained within said die housing (29).

26. The apparatus of claim 24 or 25 wherein said nozzle exterior surface includes a first axial portion (68) having a first predetermined radial extent and an axial end portion (70) having a land surface (72) including said resin outlet orifice (41) extending therethrough and having a second predetermined radial extent which is less than said first radial extent, said nozzle (31) including a tapered axial portion (74) extending between said first axial portion (68) and said axial end portion (70).

27. The apparatus of one of claims 24 to 26 wherein said nozzle (31) has a nozzle exterior surface, said nozzle exterior surface having a plurality of flutes (76) adjacent said resin outlet orifice (41) to direct said primary fiberization fluid.

28. The apparatus of claim 27 wherein nozzle (31) has a flute attack angle (H') of about 7 to 60 degrees.

29. The apparatus of one of claims 27 and 28 wherein said nozzle (31) has a flute spiral angle (G') of about 20 to 45 degrees.

30. The apparatus of one of claims 26 to 29, wherein said nozzle (31) has a frustoconical angle (F') of about 15 to 60 degrees.

31. The apparatus of one of claims 27 to 30 wherein said tapered axial portion (74) including said plurality of flutes (76) said flutes (76) extending into said land surface.

32. The apparatus of claim 31 wherein said axial end portion (70) includes a substantially cylindrical outer surface including said flutes (76).

33. The apparatus of one of claims 14 to 32 which further includes collection means (24) for receiving said fibers (22) in the form of a nonwoven web (26).

34. An apparatus according to one of claims 14 to 33 for intermittently forming fibers from a fiber forming resin further comprising:
a die assembly located within said housing including said resin chamber and on/off control means (37) for selectively interrupting flow of said molten resin from said resin outlet orifice (41).

35. The apparatus of claim 34 wherein said on/off control means includes a plunger (37) within said resin chamber having a closed position wherein said plunger (37) is in contact with said resin outlet orifice (41) for preventing flow of said molten resin from said orifice (41) and an open position wherein said plunger (37) is retracted from said orifice (41) to allow flow of said molten resin from said orifice.

36. The apparatus of claim 34 or 35 wherein said die housing (29) includes a hydraulic chamber, said plunger (37) including an end portion extending into said hydraulic chamber (96) including a piston (100) mounted thereon, said chamber including hydraulic fluid ports (104, 106) opening into said hydraulic chamber for supplying varying fluid pressure on each side of said piston (100) to reciprocate said piston (100) within said hydraulic chamber (96) to move said plunger (37) between said open and closed positions.

37. An apparatus according to one of claims 14 to 36 for forming a nonwoven web from a fiber forming resin further comprising:
a plurality of die assemblies (16) located within said housing, each die assembly (16) including a resin chamber for receiving a supply of molten fiber forming resin, each of said chambers having a resin outlet orifice (41) in fluid communication therewith for emitting said molten resin in the form of a flow, said flow extending preferably along a first axis, on/off control means (37) for selectively interrupting said flow of resin from at least one of said resin outlet orifices (41) to vary the density of said nonwoven web (26).

38. The apparatus of claims 24, 26 and 37 wherein said axial end portion (70) has preferably a substantial cylindrical outer surface having a land surface (72) and said axial end portion (70) including a plurality of flutes (76), said flutes (76) extending into said land surface (72) and preferably are situated in the cylindrical outer surface.

39. Use of the apparatus according to one of claims 37 and 38 for forming a nonwoven web of varying basis weight and/or for forming individual nonwoven webs in a continuous formation process.

## Patentansprüche

1. Verfahren zur Faserbildung aus einem faserbildenden Harz, umfassend die Schritte:
(a) Bilden eines Harzstroms aus einem Formgehäuse, welches wenigstens eine Harzauslassöffnung aufweist, wobei sich der Strom entlang einer ersten Achse erstreckt, wobei die Harzauslassöffnung sich in einer Vertiefung in dem Gehäuse befindet, und
(b) Verfasern des Harzes um Fasern zu bilden, indem man ein primär verfaserndes Fluid in komplett umgebenden Kontakt mit dem Harzstrom strömen lässt, wobei das primär verfasernde Fluid sich um die Polymerquelle windet, während es durch die Formspitze extrudiert wird, und wobei das primär verfasernde Fluid in einem Primärfluidstromwinkel zwischen etwa 15 und 60 Grad mit dem Harzstrom in Kontakt kommt, wobei der Winkel als Innenwinkel zwischen dem Schnittpunkt der ersten Achse des Harzstroms und einer Linie tangential zu dem Strom des primär verfasernden Fluids gemessen wird.

2. Verfahren gemäß Anspruch 1, welches den Schritt der weiteren Verfaserung des Harzes enthält, indem das Harz mit einem Strom eines sekundär verfasernden Fluids in Kontakt gebracht wird, einschließlich wenigstens zweier Fluidströme, die jeweils auf das Harz in einem Sekundärfluidstromwinkel zwischen etwa 1 und 45 Grad auftreffen, wobei der Winkel als Innenwinkel zwischen dem Schnittpunkt der ersten Achse des Harzstroms und einer Linie tangential zu dem Strom des Fluidstroms gemessen wird.

3. Verfahren gemäß einem der vorhergehenden Ansprüche, wobei der Harzstrom einen Schmelzdruck von weniger als oder gleich 6900 kPa aufweist.

4. Verfahren gemäß einem der vorhergehenden Ansprüche, wobei der Harzstrom eine Durchflußmenge von etwa 0,1 bis 151 Gramm pro Öffnung pro Minute aufweist, vorzugsweise von etwa 0,75 bis 38,0 Gramm pro Öffnung pro Minute.

5. Verfahren gemäß einem der vorhergehenden Ansprüche, wobei das primär verfasernde Fluid mit einer Rate von etwa 57 bis 1558 Standardlitern pro Minute fließt, vorzugsweise mit einer Rate von etwa 57 bis 708 Standardlitern pro Minute.

6. Verfahren gemäß einem der vorhergehenden Ansprüche, welches ferner den Schritt des Anwinkelns des primär verfasernden Fluidstroms enthält, so dass dieser sich um die erste Achse des Harzstroms windet.

7. Verfahren gemäß einem der vorhergehenden Ansprüche, wobei das primär verfasernde Fluid einen Druck zwischen etwa 6,9 und 317 kPa aufweist, vorzugsweise zwischen etwa 6,9 und 172 kPa.

8. Verfahren gemäß einem der vorhergehenden Ansprüche, wobei das primär verfasernde Fluid eine Temperatur zwischen etwa 137° C und 344° C aufweist.

9. Verfahren gemäß einem der vorhergehenden Ansprüche, wobei die wenigstens eine Harzauslassöffnung einen Durchmesser zwischen etwa 0,25 und 3,0 Millimeter aufweist, vorzugsweise zwischen etwa 0,5 und 1,0 Millimeter.

10. Verfahren gemäß einem der vorhergehenden Ansprüche, welches ferner den Schritt des Sammelns der Fasern in Form einer Vliesbahn enthält.

11. Verfahren gemäß Anspruch 10, wobei das Sammeln der Fasern in Form einer Vliesbahn in einem Abstand von etwa 7,5 bis 102 cm, vorzugsweise etwa 15 bis 64 cm von der Harzauslassöffnung stattfindet.

12. Verfahren zur Faserbildung aus einem faserbildenden Harz gemäß einem der vorhergehenden Ansprüche, umfassend die zusätzlichen Schritte:
(a) Pumpen eines geschmolzenen faserbildenden Harzes in eine oder mehrere Formanordnungen, wobei jede der Anordnungen eine das geschmolzene faserbildende Harz aufnehmende Harzkammer und eine Harzauslassöffnung aufweist, die zum Ausströmen des Harzes in Fluidverbindung mit der Kammer stehen, wobei jede der Anordnungen ferner einen zurückziehbaren Tauchkolben innerhalb der Harzkammer enthält, der eine geschlossene Stellung, in der der Tauchkolben mit der Harzauslassöffnung in Kontakt ist, um das Strömen des Harzes aus der Öffnung zu verhindern, und eine geöffnete Stellung aufweist, in der der Tauchkolben aus der Harzauslassöffnung zurückgezogen wird, um das Strömen des Harzes aus der Öffnung zu ermöglichen;
(b) Zurückziehen einer oder mehrerer Tauchkolben von der geschlossenen zu der geöffneten Stellung, um stoßweise Harzströme aus den Auslassöffnungen zu bilden, sobald die Tauchkolben eine geöffnete Stellung aufweisen, wobei sich die Ströme entlang individueller erster Achsen erstrecken;
(c) Unterbrechen einer oder mehrerer Harzströme durch selektives Hin- und Herbewegen des Tauchkolbens zwischen den geöffneten und geschlossenen Stellungen.

13. Verfahren gemäß Anspruch 12, wobei die Unterbrechung des Harzstroms die Bildung separater Vliesbahnen und/oder die Bildung einer separaten Vliesbahn, die Unterschiede in ihrem Flächengewicht von wenigstens 10 Prozent aufweist, zur Folge hat.

14. Vorrichtung (10) zur Faserbildung (22) aus einem faserbildenden Harz umfassend:
ein Formgehäuse (29) mit eine Harzkammer, um eine Versorgung mit geschmolzenem faserbildendem Harz zu empfangen, wobei die Kammer eine mit ihr in Fluidverbindung stehende Harzauslassöffnung (41) aufweist, um das geschmolzene Harz in Form eines Stroms auszustoßen, wobei der Strom eine erste Achse (61) definiert, wobei eine primär verfasernde Einrichtung (43) die Harzauslassöffnung (41) komplett umgibt, um das Harz in Fasern (22) zu ziehen, **dadurch gekennzeichnet, dass** die Harzauslassöffnung sich in einer Vertiefung in dem Formgehäuse befindet, und dass das primär verfasernde Fluid sich um die Polymerquelle windet, während es durch die Formspitze extrudiert wird.

15. Vorrichtung gemäß Anspruch 14, wobei die verfasernde Einrichtung eine Fluidauslassöffnung (43) in dem Formgehäuse, das den Harzstrom in der Harzauslassöffnung (41) komplett umgibt, und ein aus der Fluidauslassöffnung (43) ausströmendes primär verfaserndes Fluid enthält, um durch Verfaserung aus dem Harz Faeenm (22) zu bilden, wobei das primär verfasernde Fluid mit dem Harzstrom in einem Primärfluidstromwinkel (D') zwischen etwa 15 und 60 Grad in Kontakt kommt, wobei der Winkel als ein Innenwinkel zwischen dem Schnittpunkt der ersten Achse (61) des Harzstroms und einer Linie (51) tangential zu dem Strom des primär verfasernden Fluids gemessen wird.

16. Vorrichtung gemäß Anspruch 14 und 15, die ferner eine außerhalb der primär verfasernden Einrichtung (43) befindliche sekundär verfasernde Einrichtung (44) enthält, um ein sekundär verfaserndes Fluid bereitzustellen, welches weiterhin das Harz in Fasern (22) verfasert.

17. Vorrichtung gemäß Anspruch 16, wobei die sekundär verfasernde Einrichtung ein wenigstens zwei Fluidströme enthaltendes sekundär verfaserndes Fluid aufweist, wobei diese jeweils auf den Harzstrom in einem Sekundärfluidstromwinkel (E') zwischen etwa 1 und 45 Grad auftreffen, wobei der Winkel als ein Innenwinkel zwischen dem Schnittpunkt der ersten Achse (61) des Harzstroms und einer Linie (52) tangential zu dem Strom des Fluidstroms gemessen wird.

18. Vorrichtung gemäß Anspruch 17, wobei die wenigstens zwei Fluidströme von der Fluidauslassöffnung (43) nach außen radial und im Umfang um die erste Achse (61) symmetrisch beabstandet sind.

19. Vorrichtung gemäß einem der Ansprüche 14 bis 18, wobei das Formgehäuse (29) eine äußere Oberfläche aufweist, die eine Ebene mit der Harzauslassöffnung (41) definiert, und wobei die Fluidauslassöffnung (43) im Wesentlichen in derselben Ebene liegt, die durch die äußere Oberfläche des Formgehäuses definiert ist.

20. Vorrichtung gemäß einem der Ansprüche 14 bis 18, wobei die Fluidauslassöffnung (43) im Wesentlichen innerhalb einer Ebene (48) liegt, die durch die äußere Oberfläche des Formgehäuses definiert ist, und wobei die Harzauslassöffnung (41) innerhalb des Formgehäuses in einer Vertiefung bei einem Abstand (C') liegt, der gemessen von der Ebene (48) 5 Millimeter nicht übersteigt.

21. Vorrichtung gemäß einem der Ansprüche 14 bis 20, wobei die Harzauslassöffnung (41) einen Durchmesser von etwa 0,25 bis 3,0 Millimeter aufweist.

22. Vorrichtung gemäß einem der Ansprüche 14 bis 21, wobei die Fluidauslassöffnung (43) einen Durchmesser zwischen etwa 3 und 5 Millimeter aufweist.

23. Vorrichtung gemäß einem der Ansprüche 14 bis 22, wobei das primär verfasernde Fluid und das sekundär verfasernde Fluid durch separate Fluidzuleitungen zugeführt werden.

24. Vorrichtung gemäß einem der Ansprüche 14 bis 23, wobei das Formgehäuse (29) ferner eine darin befindliche Düse (31) umfasst, die wenigstens teilweise von einer Verfaserungsfluid-Kammer (33) umgeben ist, die in der Fluidauslassöffnung (43) endet, wobei die Düse (31) die Harzkammer und die Harzauslassöffnung (41) enthält.

25. Vorrichtung gemäß Anspruch 24, wobei die Düse (31) entnehmbar innerhalb des Formgehäuses (29) gehalten wird.

26. Vorrichtung gemäß Anspruch 24 oder 25, wobei die Düsenaußenoberfläche einen eine erste vorbestimmte radiale Ausdehnung aufweisenden ersten Axialbereich (68) und einen Axialendbereich (70) enthält, der eine Stirnfläche (72) aufweist, die die sich dahindurch erstreckende Harzauslassöffnung (41) aufweist, und der eine zweite vorherbestimmte radiale Ausdehnung aufweist, die kleiner ist als die erste radiale Ausdehnung, wobei die Düse (31) einen sich verjüngenden Axialbereich (74) aufweist, der sich zwischen dem ersten Axialbereich (68) und dem Axialendbereich (70) erstreckt.

27. Vorrichtung gemäß einem der Ansprüche 24 bis 26, wobei die Düse (31) eine Düsenaußenoberfläche aufweist, wobei die Düsenaußenoberfläche mehrere benachbart zur Harzauslassöffnung (41) liegende Rillen (76) aufweist, um das primär verfasernde Fluid zu leiten.

28. Vorrichtung gemäß Anspruch 27, wobei die Düse (31) einen Rillenangriffswinkel (H') von etwa 7 bis 60 Grad aufweist.

29. Vorrichtung gemäß einem der Ansprüche 27 bis 28, wobei die Düse (31) einen Rillenwindungswinkel (G') von etwa 20 bis 45 Grad aufweist.

30. Vorrichtung gemäß einem der Ansprüche 26 bis 29, wobei die Düse (31) einen Kegelstumpfwinkel (F') von etwa 15 bis 60 Grad aufweist.

31. Vorrichtung gemäß einem der Ansprüche 27 bis 30, wobei der sich verjüngende Axialbereich (74) die Mehrzahl von Rillen (76) enthält, wobei die Rillen (76) sich bis in die Stirnfläche erstrecken.

32. Vorrichtung gemäß Anspruch 31, wobei der Axialendbereich (70) eine die Rillen (76) enthaltende, im Wesentlichen zylindrische Düsenaußenoberfläche enthält.

33. Vorrichtung gemäß einem der Ansprüche 14 bis 32, die ferner Sammeleinrichtungen (24) zum Empfangen der Fasern (22) in Form einer Vliesbahn (26) enthält.

34. Vorrichtung gemäß einem der Ansprüche 14 bis 33 zum stoßweisen Bilden von Fasern aus einem faserbildenden Harz, ferner umfassend:
eine innerhalb des Gehäuses befindliche Formanordnung, die die Harzkammer und eine An/Aus-Steuereinrichtung (37) zum wahlweisen Unterbrechen des Stroms aus geschmolzenen Harz aus der Harzauslassöffnung (41) enthält.

35. Vorrichtung gemäß Anspruch 34, wobei die An/Aus-Steuereinrichtung einen Tauchkolben (37) innerhalb der Harzkammer enthält, der eine geschlossene Stellung, wobei der Tauchkolben (37) in Kontakt mit der Harzauslassöffnung (41) steht, um das Strömen des geschmolzenen Harzes aus der Öffnung (41) zu verhindern, und eine geöffnete Stellung aufweist, wobei der Tauchkolben (37) von der Öffnung (41) zurückgezogen wird, um das Strömen des geschmolzenen Harzes aus der Öffnung zu ermöglichen.

36. Vorrichtung gemäß Anspruch 34 oder 35, wobei das Formgehäuse (29) eine hydraulische Kammer enthält, wobei der Tauchkolben (37) einen sich bis in die hydraulische Kammer (96) erstreckenden Endbereich enthält, der einen darauf angebrachten Stempel (100) umfasst, wobei die Kammer Hydraulikfluidöffnungen (104, 106) enthält, die sich zur hydraulischen Kammer öffnen, um unterschiedlichen Fluiddruck auf jeder Seite des Stempels (100) bereitzustellen, um den Stempel innerhalb der hydraulischen Kammer (96) hin- und herzubewegen, um den Tauchkolben (37) zwischen den geöffneten und geschlossenen Stellungen zu bewegen.

37. Vorrichtung gemäß einem der Ansprüche 14 bis 36 zum Bilden einer Vliesbahn aus einem faserbildenden Harz, ferner umfassend:
eine Mehrzahl innerhalb des Gehäuses angeordneter Formanordnungen (16), wobei jede Formanordnung (16) eine Harzkammer umfasst, um eine Versorgung mit geschmolzenem faserbildendem Harz zu empfangen, wobei jede der Kammern eine mit ihr in Fluidverbindung stehende Harzauslassöffnung (41) aufweist, um das geschmolzene Harz in Form eines Stroms auszustoßen, wobei der Strom sich vorzugsweise entlang einer ersten Achse erstreckt, und eine An/Aus-Steuereinrichtung (37), um wahlweise den Harzstrom aus wenigstens einer der Harzauslassöffnungen (41) zu unterbrechen, um die Dichte der Vliesbahn (26) zu verändern.

38. Vorrichtung gemäß den Ansprüchen 24, 26 und 37, wobei der Axialendbereich (70) vorzugsweise eine im Wesentlichen zylindrische äußere Oberfläche aufweist, die eine Stirnfläche (72) aufweist, und wobei der Axialendbereich (70) mehrere Rillen (76) enthält, wobei die Rillen (76) sich bis zur Stirnfläche (72) erstrecken und sich vorzugsweise in der zylindrischen äußeren Oberfläche befinden.

39. Verwendung der Vorrichtung gemäß einem der vorhergehenden Ansprüche 37 und 38, um eine Vliesbahn mit unterschiedlichem Flächengewicht zu bilden und/oder, um individuelle Vliesbahnen in einem kontinuierlichen Bildungsverfahren zu bilden.

## Revendications

1. Procédé de formation de fibres à partir d'une résine formatrice de fibres comprenant les étapes suivantes :
(a) la formation d'un écoulement de résine à partir d'un logement de filière ayant au moins un orifice de sortie de résine, ledit écoulement s'effectuant le long d'un premier axe, dans lequel l'orifice de sortie de résine est en retrait à l'intérieur du logement de filière, et
(b) la réduction en fibres de ladite résine pour former des fibres en faisant s'écouler un fluide primaire de réduction en fibres entourant totalement ledit écoulement de résine, ledit fluide primaire de réduction en fibres s'enroulant en spirale autour de la source de polymère alors qu'il est extrudé à travers l'extrémité de la filière, et ledit fluide primaire de réduction en fibres venant en contact avec ledit écoulement de résine selon un angle d'écoulement de fluide primaire compris entre environ 15 et 60°, ledit angle étant mesuré sous la forme d'un angle intérieur entre l'intersection du premier axe dudit écoulement de résine et une ligne tangente à l'écoulement dudit fluide primaire de réduction en fibres.

2. Procédé selon la revendication 1, qui comprend l'étape supplémentaire qui consiste en la réduction en fibres de ladite résine en mettant en contact ladite résine avec un écoulement d'un fluide secondaire de réduction en fibres comprenant au moins deux courants de fluide dont chacun vient heurter ladite résine selon un angle d'écoulement de fluide secondaire compris entre environ 1 et 45°, ledit angle étant mesuré sous la forme d'un angle intérieur entre l'intersection du premier axe dudit écoulement de résine et d'une ligne tangente à l'écoulement dudit courant de fluide.

3. Procédé selon l'une des revendications précédentes, dans lequel ledit écoulement de résine s'effectue sous une pression de masse fondue n'excédant pas ou étant égale à 6 900 kPa.

4. Procédé selon l'une des revendications précédentes, dans lequel ledit écoulement de résine s'effectue à un débit d'environ 0,1 à 151 grammes par orifice par minute, de préférence d'environ 0,75 à 38,0 grammes par orifice par minute.

5. Procédé selon l'une des revendications précédentes, dans lequel ledit fluide primaire de formation de fibres s'écoule à une vitesse d'environ 57 à 1 558 litres standard par minute, de préférence à une vitesse d'environ 57 à 708 litres standard par minute.

6. Procédé selon l'une des revendications précédentes, qui comprend en outre l'étape qui consiste à donner un angle audit écoulement de fluide primaire de réduction en fibres de telle sorte qu'il s'enroule en spirale autour dudit premier axe dudit premier écoulement de résine.

7. Procédé selon l'une des revendications précédentes, dans lequel ledit fluide primaire de formation de fibres s'effectue sous une pression comprise entre environ 6,9 et 317 kPa, de préférence entre environ 6,9 et 172 kPa.

8. Procédé selon l'une des revendications précédentes, dans lequel ledit fluide primaire de formation de fibres est à une température comprise entre environ 137°C et 344°C.

9. Procédé selon l'une des revendications précédentes, dans lequel ledit au moins un orifice de sortie de résine a un diamètre compris entre environ 0,25 et 3,0 mm, de préférence entre environ 0,5 et 1,0 mm.

10. Procédé selon l'une des revendications précédentes, qui comprend en outre l'étape de collecte desdites fibres sous la forme d'une nappe non tissée.

11. Procédé selon la revendication 10, dans lequel ladite collecte desdites fibres sous la forme d'une nappe non tissée s'effectue à une distance d'environ 7,5 à 102 cm, de préférence d'environ 15 à 64 cm dudit orifice de sortie de résine.

12. Procédé de formation de fibres à partir d'une résine formatrice de fibres selon l'une des revendications précédentes, comprenant les étapes supplémentaires qui consistent en :
(a) le pompage d'une résine fondue formatrice de fibres jusque dans une ou plusieurs unités de filière, chacune desdites unités comportant une chambre à résine pour recevoir ladite résine fondue formatrice de fibres et un orifice de sortie de résine en communication de fluide avec ladite chambre pour délivrer ladite résine, chacune desdites unités comprenant en outre un plongeur rétractable à l'intérieur de ladite chambre à résine ayant une position fermée dans laquelle ledit plongeur est en contact avec ledit orifice de sortie de résine pour empêcher l'écoulement de ladite résine par ledit orifice et une position ouverte dans laquelle ledit plongeur est rétracté à l'écart dudit orifice de sortie de résine pour permettre l'écoulement de ladite résine par ledit orifice ;
(b) le retrait d'un ou plusieurs desdits plongeurs depuis ladite position fermée vers ladite position ouverte pour former par intermittence des écoulements de résine depuis lesdits orifices de sortie dont les plongeurs sont en position ouverte, lesdits écoulements se faisant selon des premiers axes individuels ;
(c) l'interruption de l'un ou de plusieurs desdits écoulements de résine en soumettant sélectivement à un cycle de fonctionnement lesdits plongeurs entre ladite position ouverte et ladite position fermée.

13. Procédé selon la revendication 12, dans lequel ladite interruption dudit écoulement de résine provoque la formation de nappes non tissées séparées et/ou la formation d'une nappe non tissée présentant des variations d'au moins 10 % de son poids de base.

14. Appareil (10) pour former des fibres (22) à partir d'une résine formatrice de fibres comprenant :
un logement de filière (29) comprenant une chambre à résine pour recevoir une alimentation en résine fondue formatrice de fibres, ladite chambre ayant un orifice de sortie de résine (41) en communication de fluide avec la chambre pour émettre ladite résine fondue sous la forme d'un écoulement, ledit écoulement définissant un premier axe (61), un premier moyen de réduction en fibres (43) entourant complètement ledit orifice de sortie de résine (41) pour étirer ladite résine en fibres (22), **caractérisé en ce que** l'orifice de sortie de résine est en retrait à l'intérieur du logement de filière, et en ce que ledit fluide primaire de formation de fibres est enroulé en spirale autour de la source de polymère alors qu'il est extrudé à travers l'extrémité de la filière.

15. Appareil selon la revendication 14, dans lequel ledit moyen de réduction en fibres comprend une lumière de sortie de fluide (43) au sein dudit logement de filière entourant complètement ledit écoulement de résine depuis ledit orifice de sortie de résine (41) et un fluide primaire de réduction en fibres émanant de ladite lumière de sortie de fluide (43) pour réduire en fibres ladite résine (22), ledit fluide de réduction en fibres venant en contact avec ledit écoulement de résine selon un angle d'écoulement de fluide primaire (D') compris entre environ 15 et 60°, ledit angle étant mesuré sous la forme d'un angle intérieur entre l'intersection du premier axe (61) dudit écoulement de résine et une ligne (51) tangente à l'écoulement dudit fluide primaire de réduction en fibres.

16. Appareil selon les revendications 14 et 15, qui comprend en outre un fluide secondaire de réduction en fibres (44) situé à l'extérieur dudit moyen primaire formateur de fibres (43) pour alimenter un fluide secondaire de réduction en fibres qui réduit davantage ladite résine en fibres (22).

17. Appareil selon la revendication 16, dans lequel ledit moyen secondaire de réduction en fibres est constitué d'un fluide secondaire de réduction en fibres comprenant au moins deux courants de fluide qui heurtent chacun ledit écoulement de résine selon un angle d'écoulement de fluide secondaire (E') compris entre environ 1 et 45°, ledit angle étant mesuré sous la forme d'un angle intérieur entre l'intersection du premier axe (61) dudit écoulement de résine et une ligne (52) tangente à l'écoulement dudit courant de fluide.

18. Appareil selon la revendication 17, dans lequel lesdits au moins deux écoulements de fluide sont symétriquement espacés radicalement et en circonférence autour dudit premier axe (61) à l'extérieur de ladite lumière de sortie de fluide (41).

19. Appareil selon l'une des revendications 14 à 18, dans lequel ledit logement de filière (29) a une surface externe qui définit un plan avec ledit orifice de sortie de résine (41) et ladite lumière de sortie de fluide (43) se trouvant sensiblement dans le même plan défini par ladite surface externe dudit logement de filière.

20. Appareil selon l'une des revendications 14 à 18, dans lequel ladite lumière de sortie de fluide (43) se trouve sensiblement à l'intérieur d'un plan (48) défini par ladite surface externe dudit logement de filière et ledit orifice de sortie de résine (41) est en retrait à l'intérieur dudit logement de filière à une distance (C') n'excédant pas 5 mm, telle que mesurée à partir dudit plan (48).

21. Appareil selon l'une des revendications 14 à 20, dans lequel ledit orifice de sortie de résine (41) a un diamètre compris entre environ 0,25 et 3,0 mm.

22. Appareil selon l'une des revendications 14 à 21, dans lequel ladite lumière de sortie de fluide (43) a un diamètre compris entre environ 3 et 5 mm.

23. Appareil selon l'une des revendications 14 à 22, dans lequel ledit fluide primaire de formation de fibres et ledit fluide secondaire de formation de fibres sont alimentés à partir d'arrivées séparées de fluide.

24. Appareil selon l'une des revendications 14 à 23, dans lequel ledit logement de filière (29) comprend en outre une buse (31) située à l'intérieur et au moins partiellement entourée par une chambre de fluide de formation de fibres (33) qui se termine dans ladite lumière de sortie de fluide (43), ladite buse (31) comprenant ladite chambre à résine et ledit orifice de sortie de résine (41).

25. Appareil selon la revendication 24, dans lequel ladite buse (31) est maintenue de manière amovible à l'intérieur dudit logement de filière (29).

26. Appareil selon la revendication 24 ou 25, dans lequel ladite surface extérieure de buse comprend une première portion axiale (68) ayant une première étendue radiale prédéterminée et une portion d'extrémité axiale (70) ayant une surface plate (72) comportant ledit orifice de sortie de résine (41) qui traverse ladite surface plate et ayant une seconde étendue radiale prédéterminée qui est inférieure à ladite première étendue radiale, ladite buse (31) présentant une portion axiale effilée (74) qui s'étend entre ladite première portion axiale (68) et ladite portion d'extrémité axiale (70).

27. Appareil selon l'une des revendications 24 à 26, dans lequel ladite buse (31) présente une surface extérieure de buse, ladite surface extérieure de buse ayant une série de cannelures (76) adjacentes audit orifice de sortie de résine (41) pour diriger ledit fluide primaire de formation de fibres.

28. Appareil selon la revendication 27, dans lequel ladite buse (31) a un angle d'attaque de cannelure (H') compris entre environ 7 et 60°.

29. Appareil selon l'une des revendications 27 et 28, dans lequel ladite buse (31) a un angle de spirale de cannelure (G') compris entre environ 20 et 45°.

30. Appareil selon l'une des revendications 26 à 29, dans lequel ladite buse (31) a un angle tronconique (F') compris entre environ 15 et 60°.

31. Appareil selon l'une des revendications 27 à 30, dans lequel ladite portion axiale effilée (74) comprend ladite série de cannelures (76), lesdites cannelures (76) pénétrant dans de ladite surface plate.

32. Appareil selon la revendication 31, dans lequel ladite portion d'extrémité axiale (70) comprend une surface externe sensiblement cylindrique comprenant lesdites cannelures (76).

33. Appareil selon l'une des revendications 14 à 32, qui comprend en outre un moyen de collecte (24) pour recevoir lesdites fibres (22) sous la forme d'une nappe non tissée (26).

34. Appareil selon l'une des revendications 14 à 33, pour former de manière intermittente des fibres à partir d'une résine formatrice de fibres constitué en outre :
d'une unité de filière disposée dans ledit logement comprenant une chambre à résine et des moyens de commande marche/arrêt (37) pour interrompre sélectivement l'écoulement de ladite résine fondue à partir dudit orifice de sortie de résine (41).

35. Appareil selon la revendication 34, dans lequel lesdits moyens de commande marche/arrêt comprennent un plongeur (37) à l'intérieur de ladite chambre à résine, ayant une position fermée dans laquelle ledit plongeur (37) est en contact avec ledit orifice de sortie de résine (41) pour empêcher l'écoulement de ladite résine fondue depuis ledit orifice (41) et une position ouverte dans laquelle ledit plongeur (37) est rétracté à l'écart dudit orifice (41) pour permettre l'écoulement de ladite résine fondue depuis ledit orifice.

36. Appareil selon la revendication 34 ou 35, dans lequel ledit logement de filière (29) comprend une chambre hydraulique, ledit plongeur (37) comprenant une portion d'extrémité s'étendant jusque dans ladite chambre hydraulique (96), portion d'extrémité sur laquelle est monté un piston (100), ladite chambre présentant des orifices de fluide hydraulique (104, 106), débouchant dans ladite chambre pour fournir une pression de fluide variable de chaque côté dudit piston (100) pour animer ledit piston (100) d'un mouvement alternatif dans ladite chambre hydraulique (96) de manière à déplacer ledit plongeur (37) entre lesdites positions ouverte et fermée.

37. Appareil selon l'une des revendications 14 à 36 pour former une nappe non tissée à partir d'une résine formatrice de fibres constitué en outre :
d'une série d'unités de filière (16) disposées à l'intérieur dudit logement, chacune desdites unités de filière (16) comprenant une chambre à résine pour recevoir une alimentation en résine fondue formatrice de fibres, chacune desdites chambres ayant un orifice de sortie de résine (41) en communication de fluide avec ladite chambre pour émettre ladite résine fondue sous la forme d'un écoulement, ledit écoulement s'étendant de préférence le long d'un premier axe, et des moyens de commande marche/arrêt (37) pour interrompre sélectivement ledit écoulement de résine à partir de l'un au moins desdits orifices de sortie de résine (41) pour faire varier la masse spécifique de ladite nappe non tissée (26).

38. Appareil selon les revendications 24, 26 et 37, dans lequel ladite portion d'extrémité axiale (70) a de préférence une surface extérieure sensiblement cylindrique ayant une surface plate (72) et ladite portion d'extrémité axiale (70) comprenant une série de cannelures (76), lesdites cannelures (76) pénétrant dans ladite surface plate (72) et de préférence sont situées dans la surface extérieure cylindrique.

39. Utilisation d'un appareil selon l'une des revendications 37 et 38 pour former une nappe non tissée de poids de base variable et/ou pour former des nappes non tissées individuelles au cours d'un procédé de formation continu.
